# EUROPEAN PATENT SPECIFICATION

(11) **EP 3 274 114 B1**
(45) Date of publication and mention of the grant of the patent: **02.09.2020**
(21) Application number: 16717719.5
(22) Date of filing: 18.03.2016
(51) Int. Cl.: B22D 19/02, B22D 19/04

(54) **A METHOD OF PRODUCTION OF LIGHT-ALLOY CASTINGS, ZONE-REINFORCED WITH METAL COMPONENTS IN THE FORM OF INSERTS, ESPECIALLY IN SAND AND PERMANENT MOULDS**
VERFAHREN ZUR HERSTELLUNG VON LEICHTLEGIERUNGSGUSSSTÜCKEN, DIE MIT METALLKOMPONENTEN IN FORM VON EINSÄTZEN ZONAL VERSTÄRKT SIND, INSBESONDERE IN SAND- UND DAUERFORMEN
PROCÉDÉ DE FABRICATION DE PIÈCES COULÉES EN ALLIAGE LÉGER, À RENFORCEMENT LOCAL PAR DES COMPOSANTS MÉTALLIQUES EN FORME DE PIÈCES RAPPORTÉES, EN PARTICULIER DANS DES MOULES EN SABLE ET PERMANENTS

(30) Priority: 24.03.2015 PL 41173315
(43) Date of publication of application: 31.01.2018
(73) Proprietor: Thoni Alutec Sp. z.o.o., 37-450 Stalowa Wola (PL)
(72) Inventor: THONI, Lothar, 37-450 Stalowa Wola (PL)
(74) Representative: Hudy, Ludwik
(86) International application number: PCT/PL2016/000030
(87) International publication number: WO 2016/153370

(56) References cited:
- EP-A2- 1 134 094
- WO-A1-97/38808
- WO-A1-2006/042350
- WO-A1-2012/041542
- GB-A- 879 287
- GB-A- 2 047 587
- GB-A- 2 073 633
- US-A- 3 815 660
- US-A1- 2012 067 537

## Description

### Clean version of description

The object of the invention is a method of producing light-alloy castings of large dimensions being zone-reinforced with metal components in the form of inserts, especially in sand and permanent moulds.

In a Polish work "Solidification of Metals and Alloys" by Zbigniew Gorny, vol. II, published in 1987 by Ossolineum Publishing House, there are known descriptions of reinforced and multi-layer castings, e.g. on p. 148 and further, there are descriptions of examples of machine components made from light alloys with metal inserts embedded in them, including pistons made from Ai-Si with embedded cast-iron inserts.

There are known methods of producing aluminum composite castings in a metal shield, e.g. PL 216806 patent, where the method consists of insertion of some powder with specific granulation made from a material of different electrical resistivity than the shield metal. After mixing with the metal, the liquid composite suspension prepared is poured either gravitationally or with the use of pressure into a mould made from a non-conductive material, representing the shape of the finished or semifinished product.

In turn, International Publication No. WO 2012/041542 A1 titled "Heat exchanger with die-cast elements and method for manufacturing the same" teaches a method for manufacturing a heat exchanger with die-cast elements, comprising a die-casting step for die-casting at least one element of a heat exchanger by means of at least one die and a positioning step for positioning at least one contoured duct inside the die, performed prior to the die-casting step. An extrusion step has been performed prior to said positioning step. The described method allows production of a heat exchanger which comprises die-cast elements that are mutually associated and have inside them at least one contoured duct witch is provided by a single metal tube.

Furthermore, International Publication No. WO 97/38808A1 titled "Composite casting having low density insert" shows a composite metallic cast article that includes a shell having a predetermined solid phase density. A non-removable insert is at least partially embedded within the shell. The insert is fabricated from a foamed metal substance having a substantially lower solid phase density than the shell. The foamed metal insert may have a layer of skin fused with the molten metal of the shell during the casting process. Tapered locating pins or other spacing elements position the insert within the mold cavity to prevent shift during the casting operation. The insert can be completely enclosed within the shell of the article, thereby expanding the design capabilities of such cast article.

In addition, from description GB 879 287 A titled "Method of encasting elongated curved pipes and pipe systems" is known a method of embedding an elongated curved hollow steel tube in a metal casting that comprises embedding the tube in a heat-insulating jacket and supporting it in a mould from the region of a bend in the tube. The tube with supports and junction is enclosed in the jacket of asbestos meal and water-glass. The jacketed tube is then placed in a pressure-casting mould and the open ends of the pipe forcibly sealed by centering members inserted by tools. During injection of the molten metal, the injection plunger is at first moved slowly and finally at an accelerated speed. The publication teaches inserting and positioning the tubes in the casting moulds using only tapering centring members, which are provided inside the mould for locating the pipes that are to be embedded and for sealing the open pipe ends to prevent penetration of the cast metal into the pipe interior.

The method of producing light-alloy castings being zone-reinforced with metal components in the form of inserts, especially produced in sand and permanent moulds, whereby the metal components in the form of inserts reinforcing the sand or permanent mould casting are most favourably mounted at the parting of the mould, and at a distance favourably not shorter than 3 mm from both the internal and the external surface, on spike- and basket-like support with the head depending on the shape of the insert, after preparing the external surfaces of the insert in the known way beforehand to increase the adhesiveness of the surface and the inserts prepared in such a way and mounted inside the casting are subject to heating to max. 600 °C to further favourably increase the adhesiveness of the surface during the filling of the mould, according to the invention, is characterized by the fact that the metal components in the form of inserts reinforcing the light-alloy casting produced in the sand or permanent casting mould are mounted in a part of the mould by embedding lengthened ends of the inserts in additional cores for stable embedding and positioning of the insert inside the mould whereby the lengthened ends are cut off and removed after casting.

The metal components reinforcing the casting, called inserts, are of different shapes and cross-sections, favourably from 0.5 mm² up to the maximum cross-sections possible to use in the casting, which are dependent on the size of the casting. The metal components reinforcing the casting, called inserts, are in a rigid form of a rod, wire or elastic, like a rope.

Moreover, the volume of the additional components reinforcing the casting - inserts embedded in a mould - cannot favourably exceed 60% of the volume of the casting being made. The application of the additional metal components reinforcing the casting, in the form of an insert in the casting, in the required volume and/or locally, aims at increasing the resistance of the casting to dynamic impacts, and it also improves the strength parameters, which has been confirmed by tests conducted on castings made in such a way. Castings with inserts, according to the invention, can be used in every field where increasing the safety levels through improving the strength is required.

This solution allows for increasing the strength parameters and the safety level maintaining the higher parameters without increasing the weight and volume of the finished component.

An example of the object of the invention is pictured in the drawing where Fig. 1 shows a view of the mould with the inserts used and Fig. 2 shows a view of the casting with an embedded rod.

The method of producing light-alloy castings, zone-reinforced with metal components in the form of inserts, especially in sand and permanent moulds, consists in the following: the metal components reinforcing the casting 1, in the form of inserts 2, in the shape of a double rod, bent to form an arc, and of a cross-section of 10 mm² in a sand casting mould 3, are most favourably mounted at the parting of the mould 3, and at a distance most favourably not shorter than 3 mm from both the internal and the external surfaces of the casting 1, with spike- and/or basket-like support 4, with the head dependent on the shape of the insert 2, after preparing the external surfaces of the insert 2 beforehand, in the known way, by fettling, shot-blasting and/or chemical cleaning, to increase the adhesiveness of the surface, and for stable embedding and positioning of the insert 2 in the sand casting mould 3. The ends of the insert 2 are inserted into additional cores 5. Moreover, the inserts 2, prepared and mounted in the casting 1 in such a way, are subject to heating to max. 600 °C for favourable additional increase of adhesiveness of the surface of the insert 2, during the filling of the mould 3. The mould 3 prepared in such a way is filled with a light aluminum alloy, and after the solidification and the knockout of the casting 1 from the mould 3 the ends of the casting 1 are cut off.

## Claims

1. A method of producing light-alloy castings being zone-reinforced with metal components in a form of inserts produced in sand and permanent moulds whereby the inserts are mounted in the moulds at a distance not shorter than 3 mm from internal and external surfaces of the casting (1) using spike-like and/or basket-like support (4) with a head dependent on shape of the insert (2) after preparing the external surfaces of the insert (2) are subject to heating to the temperature of max. 600°C to increase adhesiveness of surface of the insert (2) and the moulds are filled with a light-alloy, **characterized in that** the metal components in the form of inserts (2) reinforcing the light-alloy casting (1) produced in the sand or permanent casting mould (3) are mounted in a part of the mould (3) by embedding lengthened ends of the inserts (2) in additional cores (5) for stable embedding and positioning of the insert (2) inside the mould (3) whereby the lengthened ends are cut off and removed after casting.

2. The method according to claim 1 **characterized in that** the metal components reinforcing the casting (1), called inserts (2), mounted in the sand or permanent mould (3) are of different shapes and and have from 0,5 mm² in cross section up to the maximum cross sections possible to use in the casting (1), and the cross section of the insert (2) depends on the size of the casting (1).

3. The method according to claim 1 or 2 **characterized in that** the metal components reinforcing the casting (1), called inserts (2), mounted in the sand or permanent casting mould (3), are of a rigid form, such as that of a rod, wire and/or elastic, like a rope.

4. The method according to claim 1 or 2 **characterized in that** volume of the inserts (2) mounted in the sand or permanent casting mould (3) does not exceed 60% of volume of the casting (1) being made.

5. The method according to one of claim 1-4 **characterized in that** the light-alloy is aluminum.

## Patentansprüche

1. Ein Verfahren zur Herstellung von Gussstücken aus Leichtmetalllegierungen, die zonal mit Metallverstärkungselementen in Form von Einlagen in Sand- und Dauerformen bewehrt werden und in einem Abstand von nicht weniger als 3 mm von der Innen- und Außenflächen des Gussstücks (1) auf einer dorn- und/oder korbförmigen Unterstützung (4) mit einem Kopf je nach der Gestalt der Einlage (2) montiert werden, nach der Vorbereitung der Außenflächen der Einlage (2) auf max. 600 °C erhitzt werden, um die Haftung der Oberfläche der Einlage (2) zu erhöhen, wobei die Formen mit Leichtmetalllegierung gefüllt werden, **dadurch gekennzeichnet, dass** die Metallelemente, die das Gussstück (1) aus Leichtmetalllegierung mit Einlagen (2) in einer Sand- oder einer Dauergießform (3) verstärken, in einem Teil der Form mit zusätzlichen Kernen (5) eingebettet werden, in denen die verlängerten Enden der Einlagen (2) ausgebildet sind, um die Einlagen (2) innerhalb der Form (3) zu platzieren und zu stabilisieren, wobei die verlängerten Enden nach dem Gießen abgeschnitten und entfernt werden.

2. Das Verfahren nach Anspruch 1, **dadurch gekennzeichnet, dass** die das Gussstück (1) verstärkenden Metallelemente, die Einlagen (2) genannt werden und in einer Sand- oder einer Dauerform (3) montiert sind, unterschiedliche Gestalt haben und vorteilhaft einen Querschnitt von 0,5 mm² bis zu den maximal im Gussstück (1) verwendbaren Querschnitten aufweisen, wobei der Querschnitt der Einlage (2) von der Größe des Gussstücks (1) abhängt.

3. Das Verfahren nach Anspruch 1 oder 2, **dadurch gekennzeichnet, dass** die das Gussstück (1) verstärkenden Metallelemente, die Einlagen (2) genannt werden und in einer Sand- oder einer Dauerform (3) montiert sind, eine starre Gestalt wie ein Stab, Draht und/oder eine flexible wie ein Seil haben.

4. Das Verfahren nach Anspruch 1 oder 2, **dadurch gekennzeichnet, dass** das Volumen der zusätzlichen Verstärkungselemente, der Einlagen (2), die in einer Sand- oder einer Dauerform (3) montiert sind, 60% des Volumens des Gussstücks (1) nicht überschreiten darf.

5. Das Verfahren nach einem der Ansprüche 1-4, **dadurch gekennzeichnet, dass** die Leichtmetalllegierung Aluminium ist.

## Revendications

1. Procédé de production de pièces moulées en alliage léger à renfort de zones par des composants métalliques sous forme d'inserts produits dans des moules en sable et permanents, les inserts étant montés dans les moules à une distance non inférieure à 3 mm des surfaces internes et externes de la pièce moulée (1) en utilisant un support en forme de pointe et/ou en forme de panier (4) avec une tête qui dépend de la forme de l'insert (2) après préparation, les surfaces externes de l'insert (2) sont soumises à un chauffage à la température maximale de 600°C pour augmenter l'adhésivité de la surface de l'insert (2) et les moules sont remplis d'un alliage léger, **caractérisé en ce que** les composants métalliques sous forme d'inserts (2) qui renforcent la pièce moulée en alliage léger (1) produite dans le moule de coulée en sable ou permanent (3) sont montés dans une partie du moule (3) en encastrant les extrémités allongées des inserts (2) dans des noyaux supplémentaires (5) pour un encastrement et un positionnement stables de l'insert (2) à l'intérieur du moule (3), les extrémités allongées étant coupées et retirées après la coulée.

2. Procédé selon la revendication 1, **caractérisé en ce que** les composants métalliques renforçant la pièce moulée (1), appelés inserts (2), montés dans le moule en sable ou permanent (3), sont de formes différentes et présentent une section transversale allant de 0,5 mm² jusqu'aux sections transversales maximales possibles à utiliser dans la pièce moulée (1), et la section transversale de l'insert (2) dépend de la taille de la pièce moulée (1).

3. Procédé selon la revendication 1 ou 2, **caractérisé en ce que** les composants métalliques renforçant la pièce moulée (1), appelés inserts (2), montés dans le moule de coulée en sable ou permanent (3), possèdent une forme rigide, comme celle d'une tige, d'un fil et/ou d'un élastique, comme une corde.

4. Procédé selon la revendication 1 ou 2, **caractérisé en ce que** le volume des inserts (2) montés dans le moule de coulée en sable ou permanent (3) ne dépasse pas 60% du volume de la pièce moulée (1) en cours de réalisation.

5. Procédé selon l'une des revendications 1 à 4, **caractérisé en ce que** l'alliage léger est de l'aluminium.
